

April 30, 1929.

W. L. WRIGHT

1,711,337

CAPPING MILK BOTTLES AND OTHER CONTAINERS

Original Filed July 12, 1923



*Inventor*  
W. L. Wright

By

*Herbert B. Beck* attorney

## UNITED STATES PATENT OFFICE.

WILBUR L. WRIGHT, OF FULTON, NEW YORK.

## CAPPING MILK BOTTLES AND OTHER CONTAINERS.

Original application filed July 12, 1923, Serial No. 650,980. Divided and this application filed September 15, 1928. Serial No. 135,668.

This case constitutes a division of my application filed July 12, 1923, Ser. No. 650,980, now Patent No. 1,603,057, dated October 12, 1926; and the instant case is devoted to a particular species, under the generic invention 5 of my said patent; a species that is not specifically claimed by my patent although sufficiently disclosed thereby to enable the chemist to practice the same.

10 The object of the instant invention is to utilize my discovery that so-called insoluble soaps or what I herein term, synthetic waxes, when combined with container closure disks, constitute desirable binders, and hence my 15 invention consists in a paper or like material closure or hood cap disk that embodies a so-called insoluble soap as a binder.

Referring to the accompanying drawings, forming a part hereof:—

20 Fig. 1 shows a hood cap disk, to be molded over a container mouth, to form a hood cap or cover thereon in accordance with my invention.

Fig. 2 shows in plan a paper disk of my 25 invention, to be pressed into hood form on a container mouth, the sheet paper being impregnated throughout with the binder.

Fig. 3 more or less diagrammatically illustrates in side elevation, a bottle mouth, a 30 forming head, and in edge view a disk of Figs. 1 or 2 in heated condition to be pressed down and molded on the bottle mouth by any suitable head diagrammatically illustrated.

Fig. 4 is a side elevation of a bottle head 35 or mouth and a paper hood cap secured thereon in accordance with my invention.

Fig. 5 shows in side elevation, a paper or other sheet fibrous material cap possessing the characteristics of and embodying my 40 invention, and in skirted or flared hood form for application in such form to container mouths for securing thereon, when softened by heat, by contraction under the exterior container mouth rim.

45 In carrying out my invention, flat sheet disks 1 are punched or stamped from sheet material such as paper or other fibrous material suitable for the uses to which the completed disks are to be applied, such as exteriorly capping the mouths of containers. These flat disks 1 are of a size to form a 50 skirted or flanged cover or hood cap, such as 3, that will exteriorly cover and protect the mouth portion of a container, such as bottle 2, and fit under the shoulder formed by the

annular exterior rim 2\*, of the mouth portion thereof, or otherwise to secure the cap on the bottle mouth by contraction into a depression or under a projection at the exterior of the neck. 60

It is a characteristic of my invention, that by embodying in the disk, a binder of certain characteristics, I can form each disk of a single ply or layer of thin inexpensive fibrous material such as certain commercial papers or so-called pulp boards, without building up special material layer by layer or otherwise constructing the same in laminated or multi-ply form to structurally include therein layers of one or more materials. I 65 have discovered that a sheet of single-ply or comparatively thin flexible commercial paper of one thickness, when carrying any one or more of several binder substances, meeting certain requirements, distributed 70 throughout such paper, or if only at the portions thereof that are to perform securing or holding functions, will possess certain characteristics necessary for hood cap purposes, under my invention. For instance, 75 sheet fibrous material suitable for hood cap purposes, impregnated in whole or in part with a binder that embodies or is composed of any one of certain synthetic waxes or insoluble soaps, possesses characteristics with- 80 in the spirit and scope of my invention. 85

I find that sheet paper material that embodies any one or more of such substances as a binder remains stiff or set, at the portions treated therewith, at atmospheric or climatic 90 temperatures, and becomes soft, pliable or moldable when heated to the necessary high temperatures to fuse or melt the binder in the paper, is sanitary for use on or in connection with food products, is approximately 95 insoluble in water, is without objectionable odor when cool or set, does not attract vermin or insects, is non-poisonous, does not objectionably foul glass surfaces of the cap forming or applying head, is not seriously 100 objectionable in color, and is of quick setting characteristics.

The single ply or thin paper material disks or caps can be treated with the insoluble soap binders hereinbefore mentioned, by dipping or otherwise applying the hot liquid melted binder to the paper to thoroughly impregnate the same. I prefer to impregnate the paper or sheet fibrous material with the molten binder and drain or otherwise remove sur- 105 110

plus binder from the surface of the paper. As at present advised by experience, I wish to avoid excess exterior coatings of the binder on the surfaces of the paper but wish the 5 binder to fill or impregnate the body or interior of the paper, as the excess surface coatings are but surplusage and when the paper is heated to or above the binder-melting point such surplus surface coatings are liable to 10 flow therefrom to adjacent or contacting objects.

The paper disks 1, can be impregnated and thereby rendered normally stiff at their edge portions only, see 1<sup>a</sup>, Fig. 1, or can be rendered 15 normally stiff throughout by more or less complete impregnation, as indicated by the disk 1, of Fig. 2.

In both forms, however, the disk when softened by heating to or above the melting 20 point of the binder, is molded, shaped or pressed on the bottle mouth into hood cap form, by any suitable forming, pressing or spinning head 5, diagrammatically indicated in the drawings. The hood cap thus formed 25 on the bottle mouth from the flat disk 1 when softened by heat, has a usually flat central portion *b* (whereon usually appear certain exposed display indicia, legends or advertising) and an annular depending skirt or flange 30 *c* that is contracted at *d* under the exterior rim of the bottle mouth, and that quickly sets and becomes stiff or more or less rigid at climatic or atmospheric temperatures to secure or lock the hood cap on the bottle mouth. 35 The skirt or flange thus provides the self securing or locking portion *d* of the hood cover, and it is essential that at least the portion of the paper disk 1 that is to form this part *d* of the hood cap, be impregnated with 40 the binder.

The bottlers will purchase these flat treated paper disks, and will be equipped with proper implements or machines for molding the flat disks, when softened by heat, directly on 45 the bottle mouths to form the hood caps thereon, in such manner that said caps remain locked or secured on the bottle mouths by the stiff or rigid contracted flanges of the caps. The softened portions of the caps, quickly 50 cool to atmospheric temperatures and quickly become set and rigid so that removal of the cap preferably requires expansion, rupture or tearing of the flange thereof, although this can be accomplished by the fingers without 55 the use of special or other tools.

Paper or other sheet fibrous material impregnated with or embodying various insoluble soaps or so-called synthetic waxes, possesses the characteristics of, and are within 60 the scope of my invention. Such insoluble soaps are solids at climatic temperatures and have melting points around 270° F. more or less, and can be composed of hard high melting point quick setting waxes, among others, 65 such as Montan, carnauba, or candelilla, or

stearic acid, and other ingredients. For instance, I find that compositions about as follows are suitable for the purposes of my invention, namely:—

|                                         |          |    |
|-----------------------------------------|----------|----|
| (1) Montan wax                          | 500 g.   | 70 |
| Stearic acid                            | 270 g.   |    |
| Soda ash                                | 15½ g.   |    |
| Magnesium acetate                       | 17 g.    |    |
| Caustic aluminum solution about 37½° Bé | 50 c. c. | 75 |

For use for my purposes, this composition is mixed with paraffin oil in the proportion of about 20 parts of composition to 1 part oil.

|                                         |          |    |
|-----------------------------------------|----------|----|
| (2) Carnauba wax                        | 420 g.   | 80 |
| Stearic acid                            | 420 g.   |    |
| Magnesium acetate                       | 15 g.    |    |
| Caustic aluminum solution about 37½° Bé | 75 c. c. | 85 |

This composition is also mixed with paraffin oil in about the same proportions as where composition (1) is used.

|                                         |           |    |
|-----------------------------------------|-----------|----|
| (3) Candelilla wax                      | 160 g.    | 90 |
| Stearic acid                            | 640 g.    |    |
| Magnesium acetate                       | 10 g.     |    |
| Paraffin                                | 48 g.     |    |
| Caustic aluminum solution about 37½° Bé | 120 c. c. | 95 |

For my purpose this composition is mixed with paraffin oil in about the proportions of ten parts composition to one part oil.

The caustic aluminum solution hereinbefore mentioned was produced by employing 100 metallic aluminum and caustic soda in proportions 1 part aluminum to 10 parts soda with sufficient water to make the solution read 37½° Bé., although I do not wish to so limit my invention.

The proportions of the ingredients of the several compositions can be varied and also equivalent ingredients can be employed in each composition, and I do not wish to limit my invention to the compositions as outlined but wish to cover and include sheet material possessing the characteristics of my invention whatever insoluble soap binders suitable for the purpose, may be included or embodied therein.

In the compositions indicated caustic solutions of other metals than aluminum can be employed to form an insoluble stearate or palmitate (for example, such as lead).

Paper or other fibrous sheet material of my invention hereinbefore described possessing the characteristics substantially as pointed out, can be put on the market in various forms, and shapes for container capping and other purposes, and I do not wish to limit 125 all features of my invention to the flat disk form, hereinbefore described.

For instance, in Fig. 5, I show such sheet material of my invention in premolded, drawn or pressed into flanged, skirted or 130

- flared hood cap form, for the market. These caps 7, of Fig. 5 can be prepared for the market from the flat disks of Figs. 1 or 2, either impregnated with the binder at the 5 lower edge or securing portions of their skirts 7<sup>a</sup>, or impregnated throughout. These flared skirted caps are usually pressed or drawn by dies from commercial sheet paper such as pulp board, as hereinbefore described, and 10 then impregnated with the binder hereinbefore mentioned, as described in connection with the flat disks. Surplus or surface binder coating is preferably removed from the skirted caps, before they are ready for packing 15 and shipment.
- These skirted binder carrying caps, are flared so that they can be nested to reduce the space required for packing, and also to facilitate the application thereof to bottle mouths. 20 These flared skirted caps are softened by heat before or after they are slipped onto the bottle mouths, and while so softened, any suitable means is utilized to contract the securing impregnated portions of the cap skirts, to fasten 25 and secure the caps on the bottle mouths, by the cooling and setting thereof, as hereinbefore described in connection with the flat binder impregnated disks.
- What I claim is:
- 30 1. A sheet paper disk for bottle mouth hood
- capping having at least that portion that forms the securing part of the cap skirt, embodying an insoluble soap or synthetic wax. 35
2. A sheet paper disk for bottle mouth hood capping having at least that portion that forms the securing part of the cap skirt, embodying an insoluble soap including stearic acid and a high melting point hard wax. 40
3. A paper hood cap carrying a water-insoluble soap as a binding medium. 45
4. A paper hood cap adapted to be bound about a glass bottle head, said cap carrying a metallic-organic composition as a binder which when softened by heating will quickly set to hold the cap in place on the container. 50
5. A paper hood cap carrying as a binder a water insoluble soap and a hard wax. 55
6. A paper hood cap for a glass container carrying a binder containing a fatty acid and basic material in at least partial combination. 60
7. A paper material hood cap having its skirt provided with a binder embodying stearic acid as a major ingredient.
8. A paper hood cap carrying a water-resistant binder containing an insoluble soap. 55
- In testimony whereof I have hereunto set my hand at Fulton, N. Y., this third day of September, 1926.

WILBUR L. WRIGHT.

Patent No. 1,711,337.

Granted April 30, 1929, to

WILBUR L. WRIGHT.

It is hereby certified that the above numbered patent was erroneously issued to the inventor said "Wright", whereas said patent should have been issued to "Oswego Falls Corporation, of Fulton, N. Y., a Corporation of New York", said corporation being assignee of the entire interest in said invention, as shown by the records of assignments in this office; and that the said Letters Patent should be read with this correction therein that the same may conform to the record of the case in the Patent Office.

Signed and sealed this 28th day of May, A. D. 1929.

M. J. Moore,  
Acting Commissioner of Patents.

(Seal)

- flared hood cap form, for the market. These caps 7, of Fig. 5 can be prepared for the market from the flat disks of Figs. 1 or 2, either impregnated with the binder at the 5 lower edge or securing portions of their skirts 7<sup>a</sup>, or impregnated throughout. These flared skirted caps are usually pressed or drawn by dies from commercial sheet paper such as pulp board, as hereinbefore described, and 10 then impregnated with the binder hereinbefore mentioned, as described in connection with the flat disks. Surplus or surface binder coating is preferably removed from the skirted caps, before they are ready for packing 15 and shipment.
- These skirted binder carrying caps, are flared so that they can be nested to reduce the space required for packing, and also to facilitate the application thereof to bottle mouths. 20 These flared skirted caps are softened by heat before or after they are slipped onto the bottle mouths, and while so softened, any suitable means is utilized to contract the securing impregnated portions of the cap skirts, to fasten 25 and secure the caps on the bottle mouths, by the cooling and setting thereof, as hereinbefore described in connection with the flat binder impregnated disks.
- What I claim is:
- 30 1. A sheet paper disk for bottle mouth hood
- capping having at least that portion that forms the securing part of the cap skirt, embodying an insoluble soap or synthetic wax. 35
2. A sheet paper disk for bottle mouth hood capping having at least that portion that forms the securing part of the cap skirt, embodying an insoluble soap including stearic acid and a high melting point hard wax. 40
3. A paper hood cap carrying a water-insoluble soap as a binding medium. 45
4. A paper hood cap adapted to be bound about a glass bottle head, said cap carrying a metallic-organic composition as a binder which when softened by heating will quickly set to hold the cap in place on the container. 50
5. A paper hood cap carrying as a binder a water insoluble soap and a hard wax. 55
6. A paper hood cap for a glass container carrying a binder containing a fatty acid and basic material in at least partial combination. 60
7. A paper material hood cap having its skirt provided with a binder embodying stearic acid as a major ingredient. 65
8. A paper hood cap carrying a water-resistant binder containing an insoluble soap. 70
- In testimony whereof I have hereunto set my hand at Fulton, N. Y., this third day of September, 1926.

WILBUR L. WRIGHT.

Patent No. 1,711,337.

Granted April 30, 1929, to

WILBUR L. WRIGHT.

It is hereby certified that the above numbered patent was erroneously issued to the inventor said "Wright", whereas said patent should have been issued to "Oswego Falls Corporation, of Fulton, N. Y., a Corporation of New York", said corporation being assignee of the entire interest in said invention, as shown by the records of assignments in this office; and that the said Letters Patent should be read with this correction therein that the same may conform to the record of the case in the Patent Office.

Signed and sealed this 28th day of May, A. D. 1929.

M. J. Moore,  
Acting Commissioner of Patents.

(Seal)